

# UNITED STATES PATENT OFFICE.

HARRY A. CORBETT, OF NEW YORK, N. Y., ASSIGNOR TO BRETT PROCESS SCREEN COMPANY, INC., OF NEW YORK, N. Y., A CORPORATION OF NEW YORK.

## ART OR METHOD OF PRODUCING PHOTOGRAPHIC SCREENS FOR HALF-TONE WORK.

1,338,492.

Specification of Letters Patent. Patented Apr. 27, 1920.

No Drawing.

Application filed March 28, 1916. Serial No. 87,758.

To all whom it may concern:

Be it known that I, HARRY A. CORBETT, a subject of the King of the United Kingdom of Great Britain and Ireland, and residing at the borough of Manhattan, in the city, county, and State of New York, have invented certain new and useful Improvements in the Art or Methods of Producing Photographic Screens for Half-Tone Work, of which the following is a specification.

My invention relates to an art or method of producing photographic screen for half-tone work, and more particularly to the production of a screen of this character where- in the body of the plate and the surface thereof containing the light diffusing, refracting or projecting portions are formed of a homogeneous, integral body, by a method by which a master plate may be quickly and accurately duplicated.

Heretofore screens in general commercial use in half-tone work have been of three general types:—Ruled screens composed of a glass plate having cut therein a large number of parallel lineal depressions, which plates have been usually used in pairs, placed face to face with the depressions of one plate extending perpendicularly to those of the other and the depressions being filled with a more or less opaque substance; the metzograph screen having a number of small, independent irregularly arranged depressions of varying sizes and depths, on one face thereof produced ordinarily by a process of erosion or an etching process; and a screen produced photographically from a master upon gelatin containing a light sensitive emulsion or substance and carried by a glass plate. To these may be added a fourth type of screen such as that described in the Letters Patent of James Willard Morris, Number 1,161,824 dated November 23, 1915, wherein the operative surface of the screen is composed of gelatin so treated as to produce a large number of closely juxtaposed, minute, lens-like formations thereupon.

While the effects secured by each of the types of commercial screens referred to, differ radically from those secured by screens of any other type and the manner of handling each type of screen may differ from that of any other, these screens have in

common the characteristic that each screen of a type, must be produced entirely separately, distinctly and independently of every other screen of that type, and by the same method or steps; making exactitude in the production of a number of similar screens practically impossible. A skilled worker in the printing arts in using a screen of any particular type can secure certain artistic effects with one screen of that type which he can not secure with another screen of the same type having theoretically identical characteristics and made by identically the same method. In other words, where each screen in itself is an original piece of work in an attempt to duplicate or reproduce, a screen, various conditions may enter into the work which will result in variances in the character of the completed article, even though the work be done by the same workman, with the same tools and in the same manner as when the original was made.

By means of the method or art of my invention, I am enabled to produce a number of photographic screens for half-tone work, each of which will be an exact replica of every other, even to the most minute detail. Screens so made will have the same character of surface formation and the same degree of transparency as every other screen, the qualities of each screen being substantially identical with those of the master with the possible exception that with a master screen of one type, it may be slightly more transparent and slightly more effective in diffusing, refracting or projecting of light rays. By my improved method, a number of screens may be produced each of which may be handled by the skilled worker in the art in exactly the same manner as any other screen of the same grade, thus avoiding those difficulties resulting from the breakage of a screen now ordinarily used commercially, and the attempt to secure another screen which a worker may use under exactly the same conditions as he did the destroyed screen. This possibility growing out of my invention is of more than secondary importance, in that one of the great objections to the ordinary screen now being commercially used is that the worker becomes accustomed to a particular screen and in case of breakage of the screen, finds it necessary to

accustom himself to a new screw by reason of the fact that it is rarely that two screens are produced which have exactly the same characteristics throughout.

5 In my experiments in perfecting my invention, I have used as a master screen one embodying the characteristics described in the said Letters Patent of James Willard Morris and in describing my invention, I  
10 will refer more particularly to the method or art of reproducing this particular screen, it being understood however, that certain of the steps essential to the practice of my invention with this Morris type of screen are  
15 not essential in connection with the use of other screens as masters, or even in reproducing a screen made in accordance with my invention.

Considering the invention in its broader  
20 aspects, my improved method or art may be used for making a number of reproductions from any type of master screen wherein the control of the light rays is due to surface formations, as distinguished from variances  
25 in the tones or degree of transparency of said surface. Specifically my invention relates to the reproduction of the screen described in the Letters Patent of the said James Willard Morris.

30 In the practice of my method or art, I apply to the surface of the master plate or screen having the depressions therein, or the elevations thereon, a superficial coating of an ammoniacal solution of nitrate of  
35 silver, precipitating the silver upon said surface in the same manner as silver is precipitated upon plate glass in the manufacture of mirrors. I have found that in this manner a continuous, electro-conductive  
40 surface may be formed upon said master screen or plate preparatory to the next step of the process. I have employed silver for the coating because of the close grain of this metal and the ease with which it may  
45 be applied to the surface of the master screen or plate. Other electro-conductive substances insoluble in an electro-plating bath, may be used in lieu thereof if desired, however, although such substance must have

50 a very close grain to give satisfactory results. Gold or platinum might be used advantageously, although I have found ordinary plumbago unsuitable for this use. Ordinarily the dimensions of the depressions  
55 and elevations which must be so coated, are so small that a granular substance or a metal having a texture or grain coarser than that of silver, would not exactly reproduce the master but would introduce in the reproduction made therefrom, certain peculiarities and eccentricities which would seriously affect the operative effect of the reproduction in its use.

I have found that when coating a screen

having a gelatin surface as described in the 65 said Letters Patent of James Willard Morris, it is extremely difficult to form a superficial coating upon the entire area of the master screen or plate, by reason of the tendency of the silver when precipitated to 70 penetrate the gelatin to a depth sufficient to interrupt the continuity of the superficial metallic coating through isolated areas of the screen surface. To check this tendency, I have found it necessary to apply a water 75 insoluble coating to the surface of the gelatin portion of the screen before coating with the electro-conductive material in a manner to protect the screen from the action of the silver solution. I have found that a thin 80 coating of celluloid dissolved in ether or alcohol or other suitable solvent, will not only impart a coating to the gelatin which will protect it in the manner referred to, but that this solution apparently closes the pores 85 of the gelatin in a manner to make the reproduction of this screen more perfect as to the lens-like formations than the master screen or plate. I attribute this to the probability that, while the lens-like formations upon the surface of the gelatin of the master screen or plate are themselves minute, nevertheless, the porosity of the gelatin results in the presence upon these lens-like formations of still smaller depressions 90 which might and probably would have the effect of modifying the operative effect of some or all of the lens-like formations in their entirety.

When the protecting coating above referred to, has been applied to the gelatin surface of the master screen or plate the superficial coating of the electro-conductive material is applied in the manner above referred to.

100 After the master plate has been thus coated, I form thereon by electro-deposition, a matrix of copper or other suitable metal, exercising the ordinary precautions used in the art of electro-plating to insure uniformity in the deposition of copper or other metal upon the metallized surface of said master screen or plate.

105 When this matrix has been deposited to the required thickness, it is separated from the master screen or plate, the silver or other superficial coating of electro-conductive material adhering firmly to the metal deposit and forming a top surface, the granular characteristics of which will be those of the 115 silver instead of those of the copper. This matrix will be an intaglio reproduction of the operative surface of the master screen or plate.

120 The matrix thus formed, is used to impress the design in intaglio thereon, upon molten glass either by a pressing or a rolling process, preferably the former.

After the glass has been so formed, the under side thereof may be ground and polished to bring the product to the desired thickness and transparency and the edges 5 having been trimmed, there will remain a solid glass screen, one surface of which will have reproduced thereon all of the surface formations found in the master screen or plate. The matrix is not injuriously affected when used to press or roll glass in 10 the manner described, and the matrix having once been formed may be used repeatedly to produce a large number of glass screens, each of which will be an exact duplicate of every other.

If it be desired to reproduce one of these glass screens that surface thereof having the operative surface formations, may be coated in the manner above referred to, to provide 20 it with an electro-conductive superficial coating and the above operation may be used to accurately reproduce this reproduction without varying in any substantial detail the characteristics of the screen made from 25 this reproduction. It will be observed that when the matrix is made from a master having a glass surface provided with lens-like formations, or other means for diffusing, refracting or projecting light rays, the 30 use of the celluloid solution, or other surface coating to prevent the metal of the electro-conductive coating penetrating this surface, is unnecessary. A screen made in accordance with my invention has the characteristics 35 that the minute indentations or depressed formations therein are inclined to have rounded edges instead of ragged or sharp edges, and that the surface will be a substantially continuous surface as distinguished from one interrupted by cutting or 40 erosion. This continuity of the surface gives mechanically, a stronger screen or plate, as well as a screen wherein the absorption or diffusion of light rays by reason of 45 small surface imperfections, is reduced to a minimum. The most important result of my improved method or art is that by means thereof a number of screens having identical qualities may be produced, and that the cost 50 of producing these screens as compared with that of producing the master is lower.

I have heretofore stated that when reproducing a screen wherein the surface formations are upon gelatin, the reproduction will 55 be superior to the master because of eliminating the porosity of the lens-like formations, and a slightly greater volume of light rays are permitted to pass through the screen. In other words the homogeneous 60 glass screen will be quicker than the gelatin master from which it was developed.

While I have found that the application of the superficial coating of electro-conductive material may be satisfactorily applied

to the master screen by following the practice ordinarily used in silvering a mirror, it is not my intention to limit the invention, considered in its broader aspects to this method. I have found that the coating methods ordinarily employed in electro-typing are not adapted for use in the practice of my method or art because the granular formation of the plumbago used did not form a continuous surface such as that required in producing minute formations upon the surface of the screen and because the plumbago does not form a smooth surface coating upon the matrix made therefrom. I believe it to be necessary to secure the desired accuracy of reproduction upon the plate or glass to press the matrix against the plastic glass, because if the glass is merely flowed over the matrix it would not result in surface formations of sufficient exactitude.

I believe it to be broadly new to produce a number of screen elevations and depressions forming the operative surface thereof, from a master screen, by a duplicating method as distinguished from a repetition of the steps used in producing the master.

It is not my intention to limit the invention to the precise steps and practices herein described, nor to the use of the specific materials herein referred to, since such are used merely as means to facilitate the practice of the method or art and to secure the best results therefrom.

Having described the invention, what I claim as new and desire to have protected by Letters Patent is:—

1. The herein described method or art of making photographic screens for half tone work consisting in applying a superficial coating of electro-conductive material to a master plate or screen having a plurality of closely juxtaposed, minute surface formations thereon, said material being of a texture or grain sufficiently fine not to modify the character of said surface formations, forming a matrix by the electro-deposition of metal upon said electro-conductive surface and impressing the design appearing in intaglio upon said matrix upon plastic material.

2. The herein described method or art of making photographic screens for half tone work consisting in applying a metallic solution to the surface of a master plate or screen having surface formations thereon, precipitating the metal of said solution upon said surface, forming a matrix by the electro-deposition of metal upon said metallized surface and impressing the design appearing in intaglio upon said matrix upon plastic glass.

3. The herein described method or art of making photographic screens for half tone work consisting in applying an ammoniacal

5 solution of nitrate of silver to the surface of a master plate or screen having surface formations thereon, precipitating the silver of said solution upon said surface, forming a matrix by the electro-deposition of metal upon said silvered surface and impressing the design in intaglio upon said matrix upon plastic glass.

10 4. The herein described method or art of making photographic screens for half tone work consisting in applying a superficial coating of electro-conductive material to a master plate or screen having a plurality of closely juxtaposed, minute surface formations thereon, said material being of a texture or grain sufficiently fine not to modify the character of said surface formations, forming a matrix by the electro-deposition of copper upon said electro-conductive surface and impressing the design appearing in intaglio on said matrix upon plastic material.

15 5. The herein described method or art of making photographic screens for half tone work consisting in applying a metallic solution to the surface of the master plate or screen having surface formations thereon, precipitating the metal of said solution upon said surface, forming a matrix by the electro-deposition of copper upon said metallized surface and impressing the design appearing in intaglio upon said matrix upon plastic glass.

20 6. The herein described method or art of making photographic screens for half tone work consisting in applying an ammoniacal solution of nitrate of silver to the surface of a master plate or screen having surface formations thereon, precipitating the silver of said solution upon said surface, forming a matrix by the electro-deposition of copper upon said silvered surface and impressing the design in intaglio upon said matrix upon plastic glass.

25 7. The herein described method or art of making photographic screens for half tone work consisting in applying a water insoluble coating to the gelatinous surface of a master plate or screen having therein a multiplicity of minute surface formations, thereafter superimposing upon said water insoluble surface a superficial coating of an electro-conductive material, forming a matrix by the electro-deposition of metal upon said electro-conductive surface and impressing the design appearing in intaglio upon said matrix upon plastic material.

30 8. The herein described method or art of making photographic screens for half tone work consisting in applying a water insoluble coating to the gelatinous surface of a master plate or screen having thereon a multiplicity of minute formations, thereafter applying a metallic solution to said

35 coating, precipitating the metal of said solution, forming a matrix by the electro-deposition of metal upon said metallized surface and impressing the design appearing in intaglio upon said matrix upon plastic glass.

40 9. The herein described method or art of making photographic screens for half tone work consisting in applying a water insoluble coating to the gelatinous surface of a master plate or screen having thereon a multiplicity of minute formations, thereafter applying an ammoniacal solution of nitrate of silver to said coating, precipitating the silver of said solution, forming a matrix by the electro-deposition of metal upon said metallized surface and impressing the design appearing in intaglio upon said matrix upon plastic glass.

45 10. The herein described method or art of making photographic screens for half tone work consisting in applying a water insoluble coating to the gelatinous surface of a master plate or screen having therein a multiplicity of minute surface formations, thereafter superimposing upon said water insoluble surface a superficial coating of an electro-conductive material, forming a matrix by the electro-deposition of copper upon said electro-conductive surface and impressing the design appearing in intaglio on said matrix upon plastic material.

50 11. The herein described method or art of making photographic screens for half tone work consisting in applying a water insoluble coating to the gelatinous surface of a master plate or screen having thereon a multiplicity of minute formations, thereafter applying a metallic solution to said coating, precipitating the metal of said solution, forming a matrix by the electro-deposition of copper upon said metallized surface and impressing the design appearing in intaglio upon said matrix upon plastic glass.

55 12. The herein described method or art of making photographic screens for half tone work consisting in applying a water insoluble coating to the gelatinous surface of a master plate or screen having thereon a multiplicity of minute formations, thereafter applying an ammoniacal solution of nitrate of silver to said coating, precipitating the silver of said solution, forming a matrix by the electro-deposition of copper upon said metallized surface and impressing the design appearing in intaglio upon said matrix upon plastic glass.

60 13. The herein described method or art of making photographic screens for half tone work consisting in applying a coating of celluloid in solution to the gelatinous surface of a master plate or screen having thereon a multiplicity of minute formations whereby

a water insoluble surface is formed, thereafter applying an ammoniacal solution of nitrate of silver to said coating, precipitating the silver of said solution, forming a 5 matrix by the electro-deposition of copper upon said metallized surface and impressing the design appearing in intaglio upon said matrix upon plastic glass.

It witness whereof I hereunto affix my signature in the presence of two subscribing 10 witnesses, this 11th day of February, 1916.

HARRY A. CORBETT.

Witnesses:

JUDITH PARDEE,  
CLARICE FRANCK.